

Patented Feb. 9, 1926.

1,572,488

# UNITED STATES PATENT OFFICE.

ZAY JEFFRIES, OF SHAKER HEIGHTS, AND ROBERT S. ARCHER, OF LAKewood, OHIO,  
ASSIGNORS TO ALUMINUM COMPANY OF AMERICA, OF PITTSBURGH, PENNSYLVANIA, A CORPORATION OF PENNSYLVANIA.

## ALUMINUM-SILICON ALLOY.

No Drawing. Original application filed January 4, 1921, Serial No. 435,024. Divided and this application filed April 29, 1924. Serial No. 709,749.

*To all whom it may concern:*

Be it known that we, ZAY JEFFRIES, of Shaker Heights, and ROBERT S. ARCHER, of Lakewood, both in the county of Cuyahoga 5 and State of Ohio, have invented certain new and useful Improvements in Aluminum-Silicon Alloys, of which the following is a full, clear, and exact description.

The invention which forms the subject of 10 our present application (a division of our copending application Serial No. 435,024, filed January 4, 1921, now patent No. 1,508, 556, issued September 16, 1924) relates to the production of aluminum alloy castings, 15 particularly castings made of alloys containing silicon or copper or both, with or without other metals, and its chief object is to provide a simple and effective method which will produce light-weight castings with a 20 hitherto unobtainable combination of physical properties, especially as regards elastic limit, tensile strength and ductility. To this and other ends the invention consists in the novel method and product hereinafter 25 described.

As will be seen from the subjoined description, the invention is based upon the combination of certain steps, some of them 30 novel with us, and in part the invention resides in the discovery that certain alloys are especially susceptible to improvement by heat treatment after casting, and that certain methods of casting such alloys further 35 and peculiarly adapt them to such treatment; and in the additional discovery of temperature and duration of heat treatment in combinations appropriate to the particular alloys and method of casting involved.

With the aid of these discoveries we have 40 been able to produce castings having improved physical properties with respect to elastic limit, tensile strength and ductility to an extent hitherto unattainable, with the result that it is now possible to use 45 aluminum alloy castings for purposes for which their use has previously been impracticable.

It has been found that the addition of a 50 substantial amount of silicon to aluminum alloys very materially improves their casting qualities, thus rendering it possible to successfully and easily make castings which would otherwise be very difficult

to produce. In particular, the presence of a substantial amount of silicon enables us to 55 produce alloys having excellent casting qualities, even better than those of the well known alloy containing 8 per cent copper, with the use of only relatively small amounts of copper or zinc or both. The possibility 60 of limiting these heavy metals to amounts of say 5 per cent or less in the case of copper, and 10 per cent or less in the case of zinc, is very advantageous, both as respects the 65 strength of the resulting alloy and as respects its specific gravity. The silicon, by virtue of its lightness, offsets, in a measure, the effect of the heavy metals, copper and zinc, as well as permitting the use of the 70 heavier metals in smaller quantities. We 75 have discovered that these silicon alloys can be materially improved by an appropriate heat treatment, which may affect both the silicon and the heavy-metal constituents.

The tensile strength of commercially pure 75 cast aluminum is about 12,000 pounds per square inch and its elongation about 25 per cent. By adding varying proportions of hardening metals, particularly copper and zinc, it is possible to increase the tensile 80 strength so that the sand cast alloy will have an ultimate strength of nearly 30,000 pounds per square inch, but the elongation is thereby reduced to less than 5 per cent. By adding a very large amount of zinc the 85 tensile strength may be raised to approximately 40,000 pounds per square inch, but the elongation is reduced to almost nothing, and the alloy is very brittle. By casting 90 any of these alloys in a chill mold, the tensile strength may be increased in general by approximately 5,000 pounds per square inch and the elongation may also be increased. But it has heretofore been impossible to simultaneously produce tensile strengths of 95 over 30,000 pounds per square inch and an elongation of 8 per cent or over.

By our method, however, we have been able to extend very greatly the range of the tensile strength and elongation, and of the 100 combination of the two, so that we have obtained castings having very much higher tensile strengths than those hitherto known in the art, and yet elongations better than those at present obtained with casting alloys 105 having only moderate tensile strengths.

2  
In general, elongation decreases as tensile strength increases, but our new method enables us to produce very much better simultaneous results in both of these respects than have hitherto been possible.

It is also to be noted that the high tensile strength alloys previously known have required the presence of substantial amounts of zinc, even in many cases up to 33 per cent, and have therefore been considerably heavier than pure aluminum, while we obtain our results with an addition, in general, of not more than 5 to 10 per cent of total heavier alloying metal or metals and yet produce a casting which is not only stronger and more ductile but likewise lighter than would otherwise be obtained.

Various prior investigators have proposed to obtain castings possessing the desirable combination of high tensile strength and ductility by heat treatment of a properly made casting, but their contributions to the art have so far not led to commercially useful results. For example, the best results published prior to our work are those of Wilm, who reports having obtained chill castings with a tensile strength of about 32,000 pounds per square inch and an elongation of 5 to 7 per cent. More recently Merica and Karr have by heat treatment of an alloy containing copper and a large amount of zinc, obtained a tensile strength of 41,200 pounds per square inch but with an elongation of only 4 per cent. This alloy contained about 19 per cent of heavy alloying metals and hence had a specific gravity greater than 3. With lighter alloys, for example one containing small amounts of copper, magnesium and manganese, they obtained a tensile strength of 35,500 pounds per square inch and an elongation of 2.3 per cent. In none of the three cases mentioned above were the properties enough better than those possessed by untreated castings to justify the cost of the treatment.

Our invention involves the discovery of important reasons for previous lack of practical success along this line, and embraces a combination of old and new steps so that we are now able by means of our improved method to produce articles, cast in either sand or chill molds, having physical properties far superior to those of any such castings hitherto produced. By means of our novel method we have produced sand castings of an aluminum alloy containing 4 per cent copper and 0.2 per cent magnesium, having a tensile strength of about 50,000 pounds per square inch and an elongation of 8.5 per cent, with relatively high elastic limit; also chilled castings having a tensile strength of 54,000 pounds per square inch and an elongation of 18 per cent, with relatively high elastic limit.

65 This combination of high tensile strength

and elongation enables these castings to be used for purposes for which aluminum castings have not hitherto been suitable and for which it has been necessary to use the much heavier ferrous materials such as steel or malleable iron.

70 One example of our process comprises as its first step the preparation of an aluminum alloy containing about 3 to 5.5 per cent copper, preferably 4 per cent, with no magnesium or with magnesium up to about 0.3 per cent, the iron content in particular being as low as possible, preferably not to exceed 0.25 per cent. Iron and silicon are always present as impurities in aluminum 75 as now obtainable, and a part of our invention consists in so choosing the raw materials as to limit the iron content of the finished alloy to an amount as low as possible, preferably not over 0.25 per cent. The use of silicon in substantial amounts will be considered hereinafter.

80 The ingredients are mixed in the molten state, care being taken to avoid excessive temperatures at all stages of the melting 85 operation, and the mixture is poured into either a sand mold or a chill mold, and caused to solidify. After solidification a microscopic examination reveals masses of an aluminum-rich constituent surrounded by 90 a network of a hard, brittle constituent, which has been reported to be chiefly CuAl<sub>2</sub>. In the form of a sand-cast test bar about one-half inch in diameter the alloy has a 95 tensile strength of 18,000 to 25,000 pounds 100 per square inch with an elongation of 2.5 to 4 per cent in two inches. A chill cast test bar of the same size has a tensile strength of about 24,000 to 28,000 pounds per square 105 inch and an elongation up to 6 per cent 110 in two inches. The iron in the alloy is found both in the form of needles, reported to be FeAl<sub>3</sub>, and in a different form, apparently as a silicide of iron. The presence 115 of the iron (FeAl<sub>3</sub>) needles up to a certain 120 amount is beneficial to the strength and ductility of the alloy in the cast condition, probably due to the fact that the ordinary path of fracture in the cast alloy is through the brittle network of CuAl<sub>2</sub>, which is strengthened by the iron needles. It is found that these iron needles are very detrimental to the physical properties of the casting after the heat treatment discussed below.

125 The next step in the example of our process now being described consists in heating the castings to, and maintaining them at, a temperature of 500° to 540° C. for a period of time depending upon the results desired and the manner in which the casting was made. The principal object of heating the castings at the temperature mentioned is to cause the CuAl<sub>2</sub> in the network to go 130 into solution in the solid aluminum-rich con-

stituent. It is found that at the temperatures referred to, this CuAl<sub>2</sub> dissolves slowly, in fact surprisingly slowly. In sand castings the time necessary for maximum solution of this CuAl<sub>2</sub> may be as much as 48 hours, at the temperatures mentioned; while in chill castings, because of the finer network structure, the time for maximum solution is less—for example, 7 hours has 10 been found to be sufficient in some cases.

If the copper content exceeds the amount which is soluble in the solid state just below the freezing point of the eutectic, some of the CuAl<sub>2</sub> will remain in the network after 15 heat treatment, and the physical properties of the casting will not be as good as can be obtained with a lower copper content. In most if not all cases the best combination of physical properties results only when substantially all of the CuAl<sub>2</sub> in the network has been dissolved in the aluminum-rich constituent.

A temperature of heat-treatment high enough to fuse the eutectic, that is, the temperature of incipient fusion of the alloy, is in most cases unfavorable to the best ultimate results, and it has been found that in some instances 540° C. is too high unless the rate of heating up to that point is very slow 25 or the time of heating below that point is comparatively long.

A further result of heating the castings at the temperature mentioned is to re-dissolve any CuAl<sub>2</sub> which may have precipitated in 30 small particles within the aluminum-rich constituent rather than in the network during the previous cooling of the castings.

After the heating period the castings are 40 preferably cooled rapidly, as by quenching in water. By the above described procedure, sand castings of an alloy containing 4 per cent copper, 0.2 per cent magnesium and less than 0.25 per cent iron have been produced within a tensile strength, after aging, 45 of about 50,000 pounds per square inch and an elongation of 8.5 per cent. Chill castings have been made by the same process, of the same alloy, having a tensile strength of 54,000 pounds per square inch after aging and an 50 elongation of 18 per cent.

As stated above, quenching is preferable to slow cooling, but good results can in some cases be obtained by cooling in a current of air. A marked difference has been observed 55 between the results obtained by cooling in a current of air and those obtained by cooling in still air. Even slow cooling, however, produces improvement as compared to the cast condition, not only in the physical properties, but also in resistance to corrosion.

The physical properties of castings subjected to the treatments above referred to can 60 be further changed by artificial aging, that 65 is, by heating them, immediately after cool-

ing, to a temperature of 100° to 150° C. for a time, one hour being in many cases sufficient. As a result of such heating the tensile strength is increased and the elongation decreased, and the elastic limit is increased 70 very markedly.

The method of casting is an important factor. Thus a method producing fine grain and improved physical properties, yields 75 castings which are generally more amenable to the heat-treatment than does a casting method which produces coarse grain. For example a bar having a cylindrical test section two inches long and a half-inch in diameter, composed of alloy containing about 80 4 per cent copper and cast in a sand mold, has a tensile strength of about 18,000 pounds per square inch and an elongation of about 4 per cent. If the bar is heat-treated by our method, say at a temperature around 520° C. 85 for 24 hours, the tensile strength may be more than doubled (increasing to about 37,000 pounds per square inch) and the elongation is increased to about 12 per cent, or three times its original value. On the other 90 hand, if the bar is cast in such a manner as to cause rapid solidification, say by chill casting in an iron mold, it will have, after heat-treatment by our method, a tensile strength of about 40,000 pounds per square 95 inch, and an elongation of about 20 per cent.

In sand castings of alloys containing substantial amounts of silicon a considerable portion of the latter appears in the form of relatively large plates or needles, and in chill 100 castings the silicon is found generally in smaller particles, some of which at least are more or less rounded. The heat-treatment changes the shape and sometimes the size of the silicon particles, tending toward a more rounded form, and the improvement in physical properties produced by the heat-treatment of such alloys is due in part to this change.

The addition, to the aluminum-copper alloys, of a small amount of magnesium, say 110 0.2 or 0.3 per cent, increases the tensile strength and elastic limit, but is less favorable to ductility or elongation. Magnesium may also be added to the aluminum-silicon 115 alloys, the effect, generally, being to increase the tensile strength and diminish the elongation.

For the best results, our experience indicates that the iron content of the aluminum copper alloy should be low, but if care is taken to make the castings by the chill method, a higher percentage of iron can be used, good results being obtained with chill 120 castings containing even more than 0.4 per cent of iron. On the other hand, in the case of heat-treated sand castings, more than that amount of iron gives less advantageous physical properties. The presence 125 of the iron is evidenced by crystalline 130

4. needles, probably of the composition  $FeAl_3$ , which usually form in the network containing  $CuAl_2$ . These needles are not soluble to any considerable extent in the solid 5 aluminum alloy, and remain intact and in place while the  $CuAl_2$  is absorbed into the body of the solid-solution crystals of aluminum during heat-treatment. The iron needles tend to have a beneficial effect on the 10 physical properties of the alloy as cast, that is before heat-treatment, but after the  $CuAl_2$  in the network has been dissolved into the aluminum-rich constituent by heat-treating, the iron needles are a source of weakness, diminishing both tensile strength and 15 elongation.

The complete elimination of the iron needles is therefore highly desirable, but the complete avoidance of iron or even its 20 reduction below about 0.25 per cent is not always practicable commercially. However when silicon is present in excess of the iron the quantity of  $FeAl_3$  formed is lessened, and some of the iron combines with the 25 silicon to form what appears to be an iron silicide. We have discovered that the latter compound freezes in a form less harmful than the needles of  $FeAl_3$ . In the case of chill castings, it is found that the  $FeAl_3$  30 needles are much smaller than in the sand castings, and hence they are not so objectionable in the heat-treated casting. Since there is considerable difficulty in commercially producing aluminum free from or 35 containing less than 0.25 per cent of iron, the desired silicon-iron relationship is most advantageously obtained by adding silicon when necessary. For example, if the iron content of the aluminum ingot is 0.35 per 40 cent and the silicon 0.3 per cent, we find it advantageous to add about 0.35 per cent silicon. We have also found that the addition of a small quantity of zinc, say 0.25 per cent, improves both the tensile strength 45 and elongation of the heat-treated castings.

Chromium up to 0.5 per cent or a little more increases the tensile strength in the heat-treated casting, but reduces the elongation.

50 With regard to the limits of copper content, we have observed that up to about 2 per cent copper, nearly all the  $CuAl_2$  remains in solution upon solidification, and that beyond 5.5 per cent copper some of the 55  $CuAl_2$  usually remains out of solution even after heat-treatment. In some cases the metal can be heated above the melting point of the eutectic of  $CuAl_2$  and aluminum without impairing its physical properties 60 provided the metal is cooled to a temperature slightly below that of complete solidification and held there for some time before quenching. When substantial percentages of iron, silicon, magnesium and zinc

are present, or any of them, the higher permissible temperature is lowered.

A very important class of alloys embraced by our invention includes the use of silicon in substantial amount, say from 3 to 15 per cent. With the silicon class of alloys 70 the best results are usually obtained when the castings are made in a chill mold. For example, a chill cast test bar of an alloy containing about 10 per cent silicon and no copper showed a tensile strength around 75 30,000 pounds per square inch and an elongation of about 7.5 per cent in two inches. After heating at 560° C. for 40 hours, followed by quenching, the tensile strength was about 27,500 pounds per square inch, 80 but the elongation was found to have been increased to 21 per cent. We are therefore able to produce by our method a casting of aluminum-silicon alloy having great ductility and at the same time a tensile strength 85 twice or more than twice that of aluminum, with the further advantage of good casting qualities as mentioned above. The addition of copper to this aluminum-silicon alloy increases the tensile strength 90 enormously but decreases the elongation. Chill cast bars of an alloy containing 6 per cent silicon and 4 per cent copper, heated 45 hours at 500° to 515° C. followed by 95 quenching, showed a tensile strength as high as 42,000 pounds per square inch and an elongation of 8 per cent. In the high silicon alloys the most advantageous copper content is from 2 to 5 per cent. It should be noted that the eutectic of the 100 aluminum-silicon system melts at 570° to 580° C., which is higher than the melting point of the aluminum-copper eutectic which is at 540° C. and therefore it is not only permissible but advantageous to heat-treat the former alloys at higher temperatures—say 530° to 570° C. When copper is added to the aluminum-silicon alloys a 105 ternary eutectic may form with a melting point of about 520° C. and consequently the heat-treatment temperature should be lowered accordingly. Zinc and magnesium also lower the maximum heat-treating temperature 110 of the aluminum-silicon alloys.

Zinc can also be added to the aluminum alloys containing substantial amounts of silicon and copper or either of them. For example an alloy containing 8 per cent silicon, 10 per cent zinc and 2.5 per cent copper, gave a tensile strength of 32,300 pounds per square inch, and an elongation of 2.5 per cent in two inches in a chill cast test bar, and after heat-treatment similar to that mentioned above the tensile strength 115 was increased to over 44,000 pounds per square inch and the elongation to 7 per cent. In case only silicon and zinc are present, it is found that the heat treatment 120 125

has a less beneficial effect on the tensile strength, but the elongation is very favorably affected. For example, in an alloy containing 8 per cent silicon and 10 per cent zinc, a chill cast test bar gave a tensile strength of 29,250 pounds per square inch and an elongation of 4 per cent, whereas after heat treatment the tensile strength was 30,500 pounds per square inch and the elongation had increased to 11 per cent. It is also found that the heat-treatment can be used in conjunction with the process for improving the physical properties of these alloys by the addition of alkali metals to the molten alloy, as described in the patent of Junius D. Edwards, Francis C. Frary and Harry V. Churchill, No. 1,410,461, issued March 21, 1922, on their application Serial No. 426,796, filed November 17, 1920. For example, chill cast test bars of an alloy containing 8 per cent silicon and 10 per cent zinc, to which alkali metals were added before pouring, gave an average tensile strength of over 41,000 pounds per square inch and an elongation of 6.2 per cent in two inches. Heat-treatment reduced the tensile strength to 34,000 pounds per square inch, but increased the elongation to 14 per cent.

To obtain the best results it is desirable, in all the above mentioned aluminum-silicon alloys, to keep the iron content low, preferably below 0.6 per cent.

It is found that the coarser the grain produced in casting, the longer must the heat-treatment be continued to produce the most beneficial results. Accordingly sand casting with large cross-sectional areas require longer heating than chill castings. Usually holding at temperature for about 7 hours is sufficient for chill castings, whereas 24 hours may be necessary with sand castings.

In addition to the production of a superior grade of sand castings, permanent mold or chill castings (including die castings), the application of our invention is also most important in connection with the forging and pressing of aluminum alloys. If it is desired to produce a forging of a given shape, a casting of suitable composition, say 4 per cent copper and 0.2 per cent magnesium, is made, preferably in a chill mold, and is subjected to heat-treatment by our method to produce a starting material for forging.

In this case, instead of quenching from the heat-treatment temperature and then reheating the article to forging temperature, we find it preferable to simply cool slowly from the heat-treatment temperature to the forging temperature. The piece is then finished to size under the press or hammer, after which it is given a short heating, say at 520° C., followed by quenching.

The duration of the heat-treatment step of our method depends, in large measure, other conditions being the same, upon the degree of improvement desired in the physical properties of the casting. 70

The essential thing to be kept in mind is the relatively long time required for cast alloys in general, as compared to those rolled aluminum-copper alloys, known to the prior heat-treating art. This is caused, 75 in the case of the cast copper alloys, by the greater difficulty in getting the unbroken CuAl<sub>2</sub> network into solution in the aluminum, and in the case of the silicon alloys by the slowness of change of form of the silicon. 80 In case both copper and silicon are present in substantial quantities, time must be allowed for both of these changes to take place to the extent necessary for the desired improvement. 85

In the copper alloys containing about 4 per cent copper, for example, it is found that heating for very long periods, say 48 hours or more, at temperatures only slightly below 500° C. will not, in general, produce as good results as a five hour treatment at 520° C. In chill castings of the copper alloys it has been found that even two hours heating at 250° C. produced substantially as good results as about 22 hours at 500° C. 95 In order to reduce the time to a minimum, we prefer, if suitable temperature control is available, to use as high a temperature as can be safely employed without spoiling the castings by overheating. 100

We have also found that in the case of alloy containing substantial amounts of silicon, the effect upon the silicon particles is produced more quickly and more completely at relatively high temperatures. In these alloys, heating for about 12 hours at 520° C. produces very substantial improvement, but the time may be extended, with slight additional improvement, if desired. 105 At a temperature of 550° to 570° C. the aluminum-silicon alloys may be heat-treated with more beneficial results than can be produced at 500° C. or thereabouts. 110

It is to be understood that the invention is not limited to the specific details herein described but can be practiced in other ways without departure from its spirit. 115

We claim:

1. In the art of making aluminum alloy castings, the method comprising preparing an alloy containing substantial amounts of silicon and zinc, casting the alloy, heating the casting to a temperature slightly below the melting point of the eutectic, and maintaining such temperature until the silicon particles have been sufficiently altered to materially improve the physical properties of the cast alloy. 125

2. In the art of making aluminum alloy castings, the method comprising preparing 130

an alloy containing substantial amounts of silicon and zinc, casting the alloy and causing the silicon therein to take the form of relatively small particles in the solidified alloy, heating the casting to a temperature slightly below the melting point of the eutectic, and maintaining such temperature until the silicon particles have been sufficiently altered to materially improve the physical properties of the cast alloy.

3. In the art of making aluminum alloy castings, the method comprising preparing an alloy containing substantial amounts of silicon and zinc, chill casting the alloy whereby the silicon is caused to take the form of relatively small particles in the solidified alloy, heating the casting to a temperature slightly below the melting point of the eutectic, and maintaining such temperature until the silicon particles have been sufficiently altered to materially improve the physical properties of the alloy.

4. In the art of making aluminum alloy castings, the method comprising preparing an alloy containing 3 to 10 per cent silicon and 5 to 15 per cent zinc, casting the alloy, heating the casting to a temperature slightly below the melting point of the eutectic, and maintaining such temperature until the silicon particles have been sufficiently altered to materially improve the physical properties of the cast alloy.

5. In the art of making aluminum alloy castings, the method comprising preparing an alloy containing substantial amounts of silicon, copper and zinc, casting the alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

45 6. In the art of making aluminum alloy castings, the method comprising preparing an alloy containing substantial amounts of silicon, copper and zinc, casting the alloy, and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

7. In the art of making aluminum alloy castings, the method comprising preparing an alloy containing substantial amounts of silicon, copper and zinc, casting the alloy, heating the casting at a temperature slightly below the melting point of the eutectic until the silicon particles have been suffi-

ciently altered and a sufficient amount of the inter-granular copper-rich constituent has been dissolved to materially improve the physical properties of the cast alloy, and cooling the casting rapidly.

8. In the art of making aluminum alloy castings, the method comprising preparing an alloy containing substantial amounts of silicon, copper and zinc, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

9. In the art of making aluminum alloy castings, the method comprising preparing an alloy containing 3 to 10 per cent silicon, 2 to 5.5 per cent copper, and 5 to 15 per cent zinc, approximately, casting the alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

10. In the art of making aluminum alloy castings, the method comprising preparing an alloy containing substantial amounts of silicon, copper and zinc, chill-casting the alloy to cause the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

11. In the art of making aluminum alloy castings, the method comprising preparing an alloy containing 3 to 10 per cent silicon, 2 to 5.5 per cent copper, and 5 to 15 per cent zinc, approximately, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

12. In the art of making aluminum alloy

- castings, the method comprising preparing an alloy containing substantial amounts of silicon, copper and zinc, casting the alloy, heating the casting to a temperature slightly 5 below the melting point of the eutectic, maintaining such temperature until the silicon particles have been sufficiently altered and a sufficient amount of the inter-granular copper rich constituent has been dissolved 10 to materially improve the physical properties of the cast alloy, and re-heating the casting at a relatively low temperature to increase the tensile strength of the alloy.
13. In the art of making aluminum alloy 15 castings, the method comprising preparing an alloy containing substantial amounts of silicon, copper and zinc, casting the alloy and causing the silicon therein to take form of relatively small particles in the solidified 20 alloy, heating the casting at a temperature slightly below the melting point of the eutectic until the silicon particles have been sufficiently altered and a sufficient amount of the inter-granular copper-rich constituent 25 has been dissolved to materially improve the physical properties of the cast alloy, cooling the casting rapidly, and reheating the casting at a relatively low temperature to increase the tensile strength of the alloy.
14. As a new article of manufacture, a 30 heat-treated casting of an aluminum alloy containing zinc, and containing silicon in amount between 3 and 15 per cent, characterized by the silicon being in the form of small finely dispersed more or less rounded 35 particles and substantially devoid of large plates and needles of silicon, with consequent high tensile strength and elongation.
15. As a new article of manufacture, a 40 heat-treated casting of an aluminum alloy containing zinc and substantial amounts of
- silicon and copper, characterized by the silicon being in the form of a small finely dispersed more or less rounded particles and substantially devoid of large silicon plates or needles and of undissolved inter-granular copper-rich constituent, with consequent high tensile strength and elongation. 45
16. As a new article of manufacture, a heat-treated casting of an aluminum alloy containing zinc and silicon and a substantial amount of copper, and having a low iron content, characterized by the substantial absence of undissolved inter-granular copper-rich constituent, and having high tensile 50 strength and elongation. 55
17. As a new article of manufacture, a heat-treated casting of an aluminum alloy containing zinc and 3 to 15 per cent silicon, containing between about 2 and 5.5 per cent of copper, and having a low iron content; characterized by the silicon being in the form of small finely dispersed more or less rounded particles and substantially devoid of large plates and needles of silicon, with 60 consequent high tensile strength and elongation. 65
18. As a new article of manufacture, a heat-treated and artificially aged casting of an aluminum alloy containing zinc and substantially amounts of silicon and copper, characterized by the silicon being in the form of small finely dispersed more or less rounded particles and substantially devoid of large silicon plates or needles and of undissolved 70 inter-granular copper-rich constituent, with consequent high tensile strength and elongation. 75

In testimony whereof we hereto affix our signatures.

ZAY JEFFRIES.  
ROBERT S. ARCHER.

- castings, the method comprising preparing an alloy containing substantial amounts of silicon, copper and zinc, casting the alloy, heating the casting to a temperature slightly 5 below the melting point of the eutectic, maintaining such temperature until the silicon particles have been sufficiently altered and a sufficient amount of the inter-granular copper rich constituent has been dissolved to materially improve the physical 10 properties of the cast alloy, and re-heating the casting at a relatively low temperature to increase the tensile strength of the alloy.
13. In the art of making aluminum alloy 15 castings, the method comprising preparing an alloy containing substantial amounts of silicon, copper and zinc, casting the alloy and causing the silicon therein to take form of relatively small particles in the solidified 20 alloy, heating the casting at a temperature slightly below the melting point of the eutectic until the silicon particles have been sufficiently altered and a sufficient amount of the inter-granular copper-rich constituent 25 has been dissolved to materially improve the physical properties of the cast alloy, cooling the casting rapidly, and reheating the casting at a relatively low temperature to increase the tensile strength of the alloy.
- 30 14. As a new article of manufacture, a heat-treated casting of an aluminum alloy containing zinc, and containing silicon in amount between 3 and 15 per cent, characterized by the silicon being in the form of 35 small finely dispersed more or less rounded particles and substantially devoid of large plates and needles of silicon, with consequent high tensile strength and elongation.
15. As a new article of manufacture, a 40 heat-treated casting of an aluminum alloy containing zinc and substantial amounts of
- silicon and copper, characterized by the silicon being in the form of a small finely dispersed more or less rounded particles and substantially devoid of large silicon plates 45 or needles and of undissolved inter-granular copper-rich constituent, with consequent high tensile strength and elongation.
16. As a new article of manufacture, a heat-treated casting of an aluminum alloy containing zinc and silicon and a substantial amount of copper, and having a low iron content, characterized by the substantial absence of undissolved inter-granular copper-rich constituent, and having high tensile 55 strength and elongation.
17. As a new article of manufacture, a heat-treated casting of an aluminum alloy containing zinc and 3 to 15 per cent silicon, containing between about 2 and 5.5 per cent 60 of copper, and having a low iron content; characterized by the silicon being in the form of small finely dispersed more or less rounded particles and substantially devoid of large plates and needles of silicon, with 65 consequent high tensile strength and elongation.
18. As a new article of manufacture, a heat-treated and artificially aged casting of an aluminum alloy containing zinc and substantially amounts of silicon and copper, characterized by the silicon being in the form of small finely dispersed more or less rounded particles and substantially devoid of large silicon plates or needles and of undissolved 70 inter-granular copper-rich constituent, with 75 consequent high tensile strength and elongation.

In testimony whereof we hereto affix our signatures.

ZAY JEFFRIES.  
ROBERT S. ARCHER.

#### Certificate of Correction.

It is hereby certified that in Letters Patent No. 1,572,488, granted February 9, 1926, upon the application of Zay Jeffries, of Shaker Heights, and Robert S. Archer, of Lakewood, Ohio, for an improvement in "Aluminum-Silicon Alloys," errors appear in the printed specification requiring correction as follows: Page 5, line 19, for "November 17, 1920" read *November 27, 1920.*; same page, line 94, for "250°" read 520°; page 6, line 94, claim 9, for the misspelled word "sfficiently" read "sufficiently"; page 7, line 43, claim 15, after the word "of" strike out the article "a"; same page, line 71, claim 18, for the word "substantially" read *substantial*; and that the said Letters Patent should be read with these corrections therein that the same may conform to the record of the case in the Patent Office.

Signed and sealed this 9th day of March, A. D. 1926.

[SEAL.]

M. J. MOORE,  
Acting Commissioner of Patents.

**Certificate of Correction.**

It is hereby certified that in Letters Patent No. 1,572,488, granted February 9, 1926, upon the application of Zay Jeffries, of Shaker Heights, and Robert S. Archer, of Lakewood, Ohio, for an improvement in "Aluminum-Silicon Alloys," errors appear in the printed specification requiring correction as follows: Page 5, line 19, for "November 17, 1920" read *November 27, 1920.*; same page, line 94, for "250°" read 520°; page 6, line 94, claim 9, for the misspelled word "sfficiently" read *sufficiently*; page 7, line 43, claim 15, after the word "of" strike out the article "a"; same page, line 71, claim 18, for the word "substantially" read *substantial*; and that the said Letters Patent should be read with these corrections therein that the same may conform to the record of the case in the Patent Office.

Signed and sealed this 9th day of March, A. D. 1926.

**[SEAL.]**

**M. J. MOORE,**  
*Acting Commissioner of Patents.*